

Oct. 13, 1931.

C. P. SANDBERG ET AL

1,827,616

MANUFACTURE OF RAILWAY AND TRAMWAY RAILS

Original Filed May 29, 1929

Fig. 1.



Fig. 2.



C. P. Sandberg,  
O. F. A. Sandberg and

N. P. P. Sandberg

by *E. F. Wiedroth*  
ATTORNEY

## UNITED STATES PATENT OFFICE

CHRISTER PETER SANDBERG, OSCAR FRIDOLF ALEXANDER SANDBERG, AND NILS PERCY PATRICK SANDBERG, OF LONDON, ENGLAND, ASSIGNORS TO THE FIRM OF MESSRS. SANDBERG, OF LONDON, ENGLAND

## MANUFACTURE OF RAILWAY AND TRAMWAY RAILS

Continuation of application Serial No. 367,082, filed May 29, 1929, and in Great Britain September 29, 1928.  
This application filed June 10, 1931. Serial No. 543,478.

A rail problem which of recent years has greatly exercised the minds of railway engineers and rail manufacturers has been the defect known as "internal fissures" which 5 may be either transverse or longitudinal. These fissures develop under service by fatigue, and may ultimately result in complete and sudden fracture of the rails without warning. A rail containing these fissures 10 is sometimes described as having a "shattered zone."

We have found that one of the chief causes of these fissures or rupturing of the steel originates in a serious difference of temperature during cooling between the outside metal and the interior metal, more particularly of the big mass in the head of the rail, while the rail is cooling through a range which occurs between 500° C. and 350° C.

20 We have found that if substantial differences in temperature are avoided between the various parts of the rail, particularly between the inner and outer portions of the rail head, while the rail is cooling through 25 this range, the danger of such defects is largely obviated.

The object of the invention is to prevent or check loss of heat by radiation at a temperature when the whole section of the rail 30 is still above 500° C. but after it has passed through the critical range, so that the temperature of the whole section becomes substantially uniform and that therefore as it subsequently cools through the range 500°–350° C., the difference of temperature between any parts of the section shall be a minimum: so avoiding the setting up of internal strains when the strength of different parts of the section is not uniform.

40 Accordingly our invention comprises the idea of so controlling the cooling of the rail between 500° C. and 350° C. that no consequential differences in temperature are present while the rail is cooling through this 45 range.

More specifically our invention comprises the step of submitting the rail to equalizing conditions, before the major mass of the rail metal, or at least the head of the rail, has 50 dropped as low as 500° C. Preferably this

equalization process is instituted before a substantial or consequential portion of the metal of the head has cooled as low as 500° C.

Our invention also includes the idea of effecting a cooling following equalization of such a character that temperature differences of a consequential degree cannot develop while the rail is cooling between 500° C. and 350° C. 55

Preliminary to setting forth the invention in greater detail it may be well to first indicate the changes which occur in certain mechanical properties of rail steels, as they cool, special consideration being given to 60 those changes which take place in the range between 500° C. and 350° C.

Therefore, referring to the drawings:

Fig. 1 shows curves representing the tensile strength and ductility of two steels, 70 .91% and .55% carbon respectively which were obtained by Dupuy and published in the Journal of the Iron and Steel Institute 1921 No. 2.

The tensile strength curves show that the 75 strength of both steels on heating tends to increase up to a temperature of about 320–350° C. and then falls very rapidly.

The ductility curves show that the elongation after a slight fall at about 250° C. rises 80 rapidly up to 430° C. and then falls to about 550–580° C. and again rises.

The reverse series of changes occurs upon cooling from a high temperature.

Fig. 2 shows some results obtained during 85 the course of the investigation which led to this invention, and were obtained by the slow bending of notched bars in the Humfrey notched bar test machine, the steel containing 0.82% C. and 0.71% manganese. The 90 curves represent the maximum bending moment which the specimens withstood and the angle they bent through before fracturing. The curves are plotted from a series of tests made at varying temperatures up to 600° C. 95 The maximum bending moment falls up to a temperature of about 150° C. rises rapidly to a maximum at about 380° C. and then falls very rapidly indeed up to the maximum temperature at which tests were made. The 100

angle bent through a very similar curve, but after falling rapidly from 400° C. to 500° C. rises again as the temperature increases.

Let us consider, by way of example, the rail head of a cooling rail which has cooled to such a stage that the head temperatures are within the range 500° to 350° C. Whether this rail has cooled from the mill heat on the hot bed in the usual way or whether the cooling has been accelerated through the critical range to produce a sorbitic micro-structure, in either case there will be a substantial difference between the interior and exterior temperatures of the head.

From the diagrams of the drawings, it will be apparent that the tensile strength of the cooler outer portions of the head have a greater strength than the hotter interior portions. As the rail cools the metal contracts.

We believe that in such a rail the hotter interior contracts more rapidly than the exterior, at least under certain conditions. Now this greater contraction of the interior portions occurring while the metal of the interior is considerably weaker than the exterior furnishes just the condition to favor the production of stresses and strains in the metal which may lead to fissures and other defects of metal structure.

Curves C and D of Fig. 1 clearly indicate how the elongation of steels may vary as the temperatures change. As the temperature rises there is a falling off in the elongation to a relatively low value between 200° and 300° C. As the temperature continues to rise the elongation increases in value until the temperature has risen to from 425° to 450° C. Further rise in temperature is accompanied by a falling off in the elongation until a temperature of from 550° to 580° C. is reached after which further rise of temperature is accompanied by increase in the elongation.

It will be readily apparent from these curves that there are two ranges of temperature within which steels on heating diminish in their ductility; first, the range 200° to 300° C., commonly known as the "blue heat" or the "blue brittle" range; and, second, the range 430° to 580° C., which latter range may be conveniently designated the "secondary brittle range" to distinguish from the primary or blue brittle range. Upon cooling steels these changes in ductility will be the reverse of those just outlined. As the rail cools from 580° C. the ductility will increase until a temperature of from 450° to 430° C. is reached. Obviously the secondary brittle range varies somewhat with different conditions such as steel composition, particular conditions of the heats and the like. Curves C and D show the variations of this secondary brittle range with varying carbon contents, curve C being for a steel having .91% carbon and curve D for a steel having .55%

carbon. With rails which are cooled without observing the precautions of our invention and which, therefore, have substantial differences between the inner and outer regions of the rail head, relatively large portions of the inner hotter metal of the rail will, at certain stages of the cooling, be in a brittle state and of a relatively low tensile strength while the cooler outer regions have greater tensile strength. These conditions will greatly increase the likelihood of the development of dangerous stresses and strains. The equalization of the temperature of the rail, in accordance with our invention, before any consequential portion of the head has cooled to 500° C. will be effective to remove stresses before the major mass of the hotter interior metal of the head has dropped below this secondary brittle zone.

In addition to the stresses caused by temperature differences between inner and outer portions of the rail stresses are also produced as a result of temperature differences between different parts of the rail as it is obvious that normally the thinner portions such as the flanges and web will drop to relatively lower temperatures than the head.

But we do not wish to be limited in any way by a particular theory as to what occurs. The essential thing is that we find it to be possible to avoid serious danger of fissures and like defects by seeing to it that the rail, particularly the rail head, cools from 500° to 350° C. with but inconsequential temperature differences between the different parts of the rail, particularly the inner and outer portions.

To more fully indicate the invention, we shall now describe several illustrative embodiments thereof.

Our invention is especially useful in the production of the so-called "heat treated" rail. Rails leave the mill with temperatures between 800° C. and 1000° C. They are allowed to cool somewhat but while still above the critical range the rail is subjected to a cooling medium to effect an accelerated cooling of at least a portion of the rail head through the critical range. Preferably we employ as the cooling medium an elastic fluid as set forth in Patent No. 1,178,352; that is to say, air, atomized water or the like.

In practice we have found the following to be an effective procedure: The rail from the mill is allowed to cool, the edge of a flange being tested from time to time with a magnet. Just as soon as the edge of the flange is found to be magnetic the head of the rail is subjected to an accelerated cooling by the application thereto of atomized water, preferably atomized to such an extent as to be in a mist like condition. Air is used in effecting atomization of the water as set forth in Patent No. 1,178,352. The cooling medium therefore in this example is a mixture of air and finely divided water. By this

treatment the desired sorbitic microstructure can be secured. The extent of sorbitization of the rail head can be easily varied by varying the length of time of application.

- 5 This treatment produces very substantial temperature differentials between the inner and outer portions of the rail head. If the rail in this non-uniform temperature condition were now to cool through this zone, 10 500° C. to 350° C., there would be a substantial chance that the stresses induced in the metal would give rise to those conditions which develop into fissures and other defective metal structure.
- 15 Therefore, immediately following the accelerated cooling through the critical range, we substantially equalize the temperature of the rail and then allow the rail to cool through at least the greater part of this range 20 of temperature, (500°-350° C.), without permitting consequential differences of temperature to occur.

It is important that the rail be submitted to equalizing conditions before the temperature 25 of the major mass of metal in the head of the rail has dropped below 500° C. Preferably the equalizing operations should be begun before a substantial part of the rail head has dropped below 500° C. Accordingly, the 30 treatment with the cooling medium should not be too drastic. In the particular example of accelerated cooling here given, the atomized water is a much less drastic quench than water in its ordinary state. The length 35 of time of application is also a factor. The more drastic the action of the cooling medium chosen, the shorter the time, both factors being chosen so that the rail may be rapidly cooled yet without lowering the temperature 40 of a substantial amount of metal of the rail head below 500° C. We moderate, in other words, the accelerated cooling. Of course, in any heat treatment operation the exterior surface may be cooled to a relatively low temperature 45 but the point which we make here is that the quench should not be sufficiently drastic nor so long continued as to lower the temperature below 500° C. to a consequential depth.

50 The equalization may be effected in various ways. For example, the rail, immediately following the sorbitizing treatment, may be introduced into a furnace in which a uniform temperature is maintained. This uniform 55 temperature may be 500° C. or even somewhat higher, but we have found that it is frequently not essential, and, in many cases, not desirable for the temperature of the furnace to be so high. We have found that furnace temperatures of 425° to 450° C. may be successfully employed. When introducing the rails into a furnace having a temperature of let us say, 450° C., the rate of cooling of the rail will immediately be greatly reduced, and the con- 60 duction of heat from the hotter interiors will

quickly bring about a condition of substantial equalization. As the temperature of no substantial part of the metal is below 500° C. upon being put in the furnace, and as the interior portions are at considerably higher temperatures substantial or approximate equalization will be effected at rail temperatures not substantially less than 500° C.; actually, in most cases at temperatures somewhat above.

75 Following equalization the rail is allowed to cool. The cooling operation should be under control to prevent consequential temperature differentials developing before the temperature has dropped to 350° C. This 20 controlled cooling may be effected in various ways. The rails may cool under shelters of one sort or another to protect them from draughts and from too rapid radiation of heat from the rails, or unduly rapid losses of heat 35 by convection or conduction. These shelters may be of more or less varied character. They may take the form of hoods which are adapted to move over the rail on the hot bed; or stationary hoods on the hot bed beneath which 90 the rails may be moved. They may be mere "lean tos" over the hot bed.

In some circumstances special shelters may be entirely dispensed with. By stacking or "bunching" the rails cooling may be sufficiently retarded to prevent damaging differentials of temperature being produced during the temperature drop to 350° C. Under certain conditions the equalized rail may cool on the hot bed without special protection or manipulation. If the situation is free from draughts and weather exposure, and weather conditions are favorable, the unprotected rail may cool down to 350° C. without consequential temperature differentials. The important thing is that the rail be freed from substantial differentials of temperature and that the cooling rail be not allowed to develop consequential differences during the cooling to 350° C.

710 While our invention is especially useful in connection with the heat treatment of rails because of the fact that the accelerated cooling of the rail necessarily introduces more or less marked differentials of temperature yet 115 our invention is of definite utility in the manufacture of ordinary rails. In cooling rails in the usual way on the hot bed we have found very decided temperature differences to occur between the thicker and thinner parts 120 of the rail, and between the inner and outer portions especially of the head. In this case, as with the heat treated rail, there is the same tendency to produce defective metal structure because of the stresses which are produced as 125 a result of substantial differentials of temperature while the rail is cooling from 500° C. to 350° C.

The rail is allowed to cool in the normal way on the hot bed until the metal has cooled 130

through the critical range. Then at some time before any substantial part of the rail has dropped to 500° C., the rail is subjected to conditions which bring about at least an approximate equalization of the temperatures of the rail which is then allowed to cool to 350° C. without permitting consequential temperature differentials to develop while cooling through such range. It will be noted that while substantial equalization is effected while the rail metal is not lower than 500° C., the temperature of the rail metal should not be above the critical range as retarded cooling through such range will produce undue softness of the metal.

Equalization and control of cooling may be accomplished in the manner already outlined with a heat treated rail. We have found the following to be especially effective and convenient in the handling of the rail not heat treated. The rail after having cooled through the critical range but while still at 500° C. or higher is placed under a hood of a material which is a poor conductor of heat. This retards the cooling sufficiently so that a condition of approximate equalization is soon reached. The rails may be allowed to remain under this hood until they have cooled to 350° C. after which they are removed therefrom and allowed to cool in the ordinary way on the hot bed.

A variation of this method of treatment may be to employ a hood over the rails, which hood may be furnished with means for supplying heat in addition to that received from the rails and the rails allowed to remain within its protection until substantial equalization of temperature is effected after which the rails may be removed therefrom and allowed to cool in the regular way on the hot bed with or without a shelter protection of some sort to prevent the appearance of substantial temperature differentials before the rail has reached 350° C. Methods such as here indicated for the ordinary rail may also be applied to the heat treated rail.

Obviously when shelters or equivalent protective means are used to retard the cooling through the range 500°-350° C. the rails may be removed therefrom after they have cooled to 350° C., or the rails may be left within them until the rails have cooled to still lower temperatures, or cooled completely.

Where we use the expressions "equalization" or "substantial" equalization of temperature in the claims, we do not intend to limit the process to obtaining an absolute uniformity of temperature of the rail. We may attain such a uniformity. We may, for example, put the rail in an equalizing furnace maintained at a constant temperature, and keep the rail there until the temperature has become uniform. On the other hand, however, we may merely reduce the rate of cool-

ing sufficiently to obtain a condition of approximate equalization, the rail then not being absolutely uniform in temperature at any stage of cooling but nevertheless being free from substantial or consequential differences of temperature while cooling through the temperature range 500° C. to 350° C.

Where we use the expression "accelerated cooling" we intend to distinguish from the ordinary cooling which takes place under ordinary conditions. We intend to cover that type of cooling in which the rate of cooling is greater than would take place except by the use of means or media for increasing such rate. By the expression "accelerated cooling" we intend to cover that increased cooling rate through the critical range of sufficient to substantially modify the micro-structure of the metal, and in particular that type of cooling which we employ for the purpose of securing a micro-structure ultimately sorbitic in character.

Having thus described our invention what we claim as new and desire to secure by Letters Patent is:

1. In a process for treating a rail, the steps of subjecting at least a portion of the rail to an accelerated cooling through the critical range and then before any consequential portion of the metal of the rail head has cooled to 500° C. subjecting the rail to temperature equalizing conditions.

2. In a process for treating a rail, the step of subjecting a cooling rail to temperature equalizing conditions before any consequential portion of the metal of the rail head has cooled to 500° C. but after the rail has cooled below the critical range.

3. In a process for treating a rail, the step of gradually cooling the rail between 500° C. and 350° C. to avoid consequential differences in temperature in the rail after the rail has cooled through the critical range.

4. In a process for treating a rail, the steps of subjecting at least a portion of the rail to an accelerated cooling through the critical range and then subjecting the rail to temperature equalizing conditions before the major mass of the head of the rail has dropped to 500° C.

5. In a process for treating a rail, the step of subjecting a cooling rail to temperature equalizing conditions after the rail has cooled through the critical range but before the major mass of the head has cooled to 500° C.

6. In a process for treating a rail, the steps of subjecting at least a portion of the rail to an accelerated cooling through the critical range but moderated to avoid cooling the major mass of the head of the rail below 500° C. and immediately subjecting the rail to temperature equalizing conditions.

7. In a process of cooling a rail from the mill heat, the steps of subjecting the rail to temperature equalizing conditions before any

consequential portion of the metal of the rail head has cooled to 500° C. but after at least a substantial part of the metal of the head has dropped below the critical range and then 5 gradually cooling the rail under conditions to prevent any consequential temperature differences therein between 500° C. and 350° C.

8. In a process for treating a rail, the steps of accelerating the cooling through the critical range and retarding the cooling through 10 the range of temperature 500° C. to 350° C.

9. In a process for cooling a rail, the steps of cooling the rail in the normal way through the critical range and retarding the cooling 15 through the range of temperature 500° C. to 350° C.

10. In a process for treating a rail, the steps of accelerating the cooling of at least a portion of the head metal through the critical range, and then subjecting the rail to temperature equalizing conditions before the major mass of the head of the rail has cooled below the secondary brittle range.

Signed at London, England, this 29th day 25 of May, 1931.

CHRISTER PETER SANDBERG.

OSCAR FRIDOLF ALEXANDER SANDBERG.

NILS PERCY PATRICK SANDBERG.

30

35

40

45

50

55

60

65